

(No Model.)

2 Sheets—Sheet 1

A. EVRARD.

HARDENING AND TEMPERING ARMOR PLATES, &c.

No. 387,712.

Patented Aug. 14, 1888.



Attest,  
Jas. R. McCathran,  
Clement Smallwood.

Inventor:  
Alfred Evrard,  
By. A. P. L. R.  
Atty.

(No Model.)

2 Sheets—Sheet 2.

A. EVRARD.

HARDENING AND TEMPERING ARMOR PLATES, &c.

No. 387,712.

Patented Aug. 14, 1888.

Fig. 4



Fig. 5



Fig. 6



Attest,  
Jas. K. McCaffrey,  
Clement Smallwood.

Inventor:  
Alfred Evrard,  
By *Alfred Evrard*  
Atty.

# UNITED STATES PATENT OFFICE.

ALFRED EVRARD, OF PARIS, FRANCE, ASSIGNOR TO THE COMPAGNIE ANONYME DES FORGES DE CHATILLON ET COMMENTRY.

## HARDENING AND TEMPERING ARMOR-PLATES, &c.

### SPECIFICATION forming part of Letters Patent No. 387,712, dated August 14, 1882.

Application filed September 18, 1886. Serial No. 213,899. (No specimens.) Patented in France June 30, 1886, No. 117,112; in England August 24, 1886, No. 10,823, and in Italy September 18, 1886, XL, 350.

*To all whom it may concern:*

Be it known that I, ALFRED EVRARD, of Paris, in the Republic of France, have invented certain new and useful Improvements 5 in Hardening or Tempering Armor-Plates, Cannon-Tubes, and other Large Objects of that Order, (for which improvements Letters Patent have been granted in Great Britain, No. 10,823, dated August 24, 1886; in France, No. 117,112, dated June 30, 1886, and a certificate of addition thereto, dated July 20, 1886, and in Italy, Vol. 40, No. 350, dated September 18, 1886,) of which the following specification is a full, clear, and exact description.

The invention relates to the hardening or tempering of armor-plates and other pieces of armor for ships or fortifications of all kinds, cannon-tubes, breech-pieces, hoops, projectiles, cylinders for rolling, axles, rings, iron plates, and other large objects of that order.

In tempering, as is well known, the effect of plunging the hot metallic object to be tempered into the comparatively cold tempering-bath is, first, to reduce with more or less suddenness the temperature of the outside, which in turn abstracts the heat from the inner portions; and the tendency of this successive cooling is to cause unequal contractions in the

mass, which put it under stress or strains that are apt to weaken the strength of the object, to warp it, and to cause ruptures therein. It is also known that the effect of tempering is, or has been, different in the case of large ob-

35 jects from what it is when applied to small objects, for not only is there greater liability to the production of injurious or destructive strains and ruptures, owing to the greater inequality in the contraction of different por-

40 tions of the mass, but it is also the fact that the tempering action in small objects pervades the mass, while in large objects it is, or has heretofore been, confined, comparatively speaking, to the surface.

45 I am aware that heretofore the tempering of armor-plates, cannon-tubes, and other objects of that order has been effected in oil; but this process is thought to be objectionable for several reasons. It is not only liable to warp the

steel, but sometimes causes the surface to crack, and, since the oil is not a good conductor of heat, there may arise differences of temperature in different parts of the bath, which would cause unequal tempering and increase the dangers from unequal contraction. 55 Moreover, since the oil cannot be heated above a comparatively low temperature, the tempering necessarily takes place at a comparatively low temperature, which necessity has heretofore restricted the choice of the metal to be used for the tempered objects in the matter of hardness, because of the excessive danger of fracture which would exist with very hard metal; and, since the oil is decomposed when exposed to a high heat, it results that the surface of the object is subjected to a much more sudden lowering of temperature than the inner parts, for the object almost instantly decomposes the oil in contact therewith, whereas the inner parts must await the slow action of conduction. It has also been proposed to temper armor-plates in water; but this process has not been employed to the extent of the oil-tempering, if at all. The difficulties before mentioned, or some of them, are or 75 would be encountered in even greater degree.

I have discovered that armor-plates, cannon-tubes, and other large objects of that order can be tempered in molten-metal baths with great advantage over the use of oil or other non-metallic baths, and I have also determined how such tempering can usefully be carried on. The molten metal, being of good conductivity, maintains an equality of temperature in all parts of the bath, and, as it may be raised to a very high temperature, the surfaces and angles can be maintained to the end of the tempering operation at such a high temperature that the object, even when of very hard steel, will support without danger the strains and stresses which the tempering develops. Moreover, the molten metal, not being decomposed or vaporized at the temperatures to which it is exposed, abstracts the heat from the surface in a more gradual and uniform manner and more nearly analogous to the abstraction of the heat from the interior of the object, for when the hot armor-plate,

cannon tube, or other object of that order is immersed in the molten-metal bath the outside particles of such object part with their heat by conduction to the adjacent particles 5 of the molten metal and raise their temperature to a degree depending upon the relative specific heats and similar conditions, and a sufficiently rapid yet regular and even interchange of heat by conduction then takes place 10 from the interior of the object to the outside thereof, from the outside of the object to the molten metal in contact therewith, and from this molten metal to the outer parts of the bath, whereas when a similar object is immersed 15 in oil it cannot raise the temperature above a certain point, the oil in contact with the object to be tempered is decomposed, and thus nearly instantaneously reduces the temperature of the outside of the object by absorption 20 of the heat energy in converting the liquid into gas or vapor, and the conduction of the heat takes place in the bath with comparative slowness. It will therefore be seen that the mutual action of the tempering-bath 25 and the article to be tempered upon each other is different in the case of metal baths from what it is in the case of oil-baths, the actual tempering-heat in the former case being the resultant of the gradual imparting of heat from 30 the object to be tempered to the metal bath until a condition of equilibrium is established, and being variable indefinitely within wide limits, and therefore capable of adaptation and regulation, and the tempering action being 35 due to a comparatively prolonged conduction of heat, whereas in the latter case (*i. e.*, with oil-baths) the tempering heat is fixed by the decomposing temperature of the oils, and the tempering is effected to a very considerable 40 extent, if not mainly, by an abstraction of heat, due to the conversion of liquid into gas or vapor and not simply to conduction.

In tempering small objects in molten-metal baths, as has heretofore been effected, the mutual action of the bath and the object to be 45 tempered are also essentially different from the tempering of armor-plates, cannon-tubes, and other objects of that order, for with small objects the tempering is effected practically in 50 an instant without any prolonged conduction of heat through the mass of the object to be tempered and of the bath and without raising the temperature of the molten-metal bath as a whole or in the part in contact with the object 55 to any considerable extent. This instantaneous tempering of small objects is due to the fact that all the particles of such objects lie on or in immediate proximity to the surface, and therefore are practically all cooled at once; 60 and the practical constancy in the temperature of the bath is due partly to the fact that its mass is large as compared to the mass of the object to be tempered, but also to the great surface of the article as compared with its 65 mass, so that a sufficient mass of the molten metal is in immediate proximity to the said

article to absorb the heat without a material rise in temperature.

I have discovered that for tempering armor-plates, cannon-tubes, and other articles of that order it is not necessary to employ a large bath of molten metal, but that a small bath as compared with the mass of the article to be tempered will suffice—say a bath of molten lead in weight equal to about three or four times the object to be tempered—although the invention is not restricted to any precise volume for the bath.

In practically carrying the invention into effect, I heat the object to be tempered to, say, 80 cherry-red or orange-yellow, and immerse it wholly (or partially, if a partial tempering only is required) in a bath of lead heated to about four hundred degrees (400°) centigrade, and I keep it therein until it has attained 85 throughout a temperature uniform with that of the molten metal. It may be retained there-in until it and the metal bath have cooled 90 nearly to the melting point of the metal of the bath.

In order to immerse the object to be tempered in the molten metal, force must be applied in consequence of the greater specific gravity of the said molten metal, thus giving a tempering under a pressure exceeding that 95 produced in tempering in oil or other non-metallic liquids. One advantage of such pressure is that it is distributed over the surface of the object and tends to prevent warping.

My invention or discovery is applicable to 100 pieces of iron or steel of any degree of softness or hardness, rolled or forged, or simply cast, or of cast-iron, or finally of a mixed or compound nature resulting from the association 105 of some of the preceding.

It specially covers the tempering of armor-plates, cannon-tubes, and other large objects, of that nature in a bath of molten metal of a 110 volume readily comparable with the mass of the object to be tempered, particularly a bath of molten lead of about three or four times the weight of the object to be tempered by heating the said object to about cherry-red or orange-yellow, and forcing it while thus hot under the molten metal, and allowing it to remain under pressure until it is of the temperature of the bath, with or without permitting the object and the bath to cool nearly to the melting point of the bath metal; but it will be understood that the conditions are variable 115 according to the nature, the form, and dimensions of the object to be tempered, the degree of temper to be attained, and other details, which those skilled in the art of tempering will be enabled to effect without further description, and that the main principle of the invention consists in the discovery that armor-plates, 120 cannon-tubes, and other large objects of that order can be effectively and advantageously tempered or hardened, not only superficially, but interiorly, through the abstraction of heat 125 from the highly-heated object by a compara-

tively prolonged conduction from the surface of the object to be tempered to the molten metal of the bath in contact therewith, and through the mass of such object and of the 5 said molten metal under which it is forced and held. This principle, it is believed, has never been employed heretofore.

For carrying out my new tempering process I have devised an apparatus which also forms 10 part of my invention or discovery, and which consists, essentially, of two furnaces of appropriate size, each provided with means for heating, and one of them containing a bath of molten metal, and being also provided with 15 means for forcing and holding the specifically-lighter objects to be tempered under the molten metal, and, in connection with such furnaces, of mechanical appliances—such as lifts and trucks—for conveying the armor-plates, 20 cannon-tubes, and other large objects of that order from the preliminary heating-furnace to the furnace containing the metal bath.

Heretofore a preliminary heating-furnace and a tempering-bath in proximity thereto 25 have had combined therewith mechanical appliances for carrying armor-plates or cannon-tubes from the heating-furnace to the bath and for lowering them therein; but the bath was of a non-metallic liquid, oil, or water, and 30 there was no means for heating the bath, and none for forcing the objects to be tempered into a specifically-heavier bath and keeping them submerged, both of which means are essential to my new apparatus.

35 The apparatus may be modified in various ways according to the nature, form, and dimensions of the objects to be tempered, the mode of heating employed, the conditions of the ground where the works are built, and so on. 40 In the accompanying drawings, which form part of this specification, two types of apparatus constructed in accordance with the invention are represented.

Figure 1 is a vertical section on line A B, 45 Fig. 3, of apparatus for tempering armor-plates; Fig. 2, a plan, the furnace containing the metal bath being uncovered, and Fig. 3 a horizontal section on line C D of Fig. 1. Fig. 4 is a side elevation of apparatus for tempering the tubes or barrels of cannons; Fig. 5, a 50 vertical longitudinal section of the same; and Fig. 6, a horizontal section taken between the furnace and the truck, whereby the pieces in tempering are moved from one furnace to the other.

55 The type of apparatus shown in Figs. 1, 2, and 3 will first be described.

An armor-plate of steel or other metal is heated by the fires N in a furnace, L, and is then 60 transferred to a second furnace, M, containing the metallic bath. A bath of lead is especially suitable. The bath is brought to suitable temperature by the gases from the furnace L, the heat being regulated by the dampers P and Q, which allows more or less of the gases 65 from the furnace L to enter the furnace M.

The arched tops of the furnaces are mounted on wheeled carriages, so that the interiors can be exposed, when desired, in tempering.

The armor-plate, having been brought to a 70 high temperature, determined by the nature of the metal, and which may be, for example, a cherry-red or orange-yellow, is placed in the lead bath, whose volume and temperature may also vary with the nature of the armor-plate, 75 its volume, the degree of temper desired, and the final temperature of equilibrium to be obtained.

In certain cases a weight of lead equal to three or four times that of the piece and an 80 initial temperature of four hundred degrees (400°) centigrade, for example, are suitable. The total immersion of the armor-plate is obtained by loading or by some other means. In certain cases the armor-plate may be tempered 85 only for a part of its thickness. The armor-plate is not withdrawn from the metallic bath until it is judged that all its parts have an equal temperature with the bath, and its withdrawal can be delayed until the temperature has fallen to within a little above the melting-point of the bath metal. In the case of the apparatus shown in Figs. 4, 5, and 6 for cannon-barrels the arrangements are somewhat different.

90 A is a vertical furnace having fire-grates C at different points in its height, which permit a regular temperature to be obtained in heating the tubes to be tempered.

95 B is the vessel containing the metallic bath. 100 This vessel is of metal, soldered, to prevent the leakage of the bath liquid. This vessel is heated externally by means of a fire-place, D, the flames from which circulate spirally around the vessel. In the bottom of the vessel is 105 fixed a pulley, I, around which moves a drag-chain for insuring the immersion of the tube in the tempering-bath. The chain is drawn upon by means of a piston moving in the hydraulic cylinder F. The lifting of the tube is 110 effected by means of a wheeled truck, K, running on the bridge H. The lifting-chain is drawn upon by means of a hydraulic cylinder, E, a system of pulleys being employed to accelerate the movement.

115 The translation or horizontal movement of the truck is obtained by means of a third hydraulic cylinder, G. The piston of this cylinder terminates in a rack, R, which engages the pinion S, having its shaft journaled in the 120 frame work of the apparatus, so that when said piston and rack R are raised the pinion S is turned in one direction, and when they are lowered the pinion is turned in the opposite direction. On the shaft of pinion S is a drum, 125 over which runs the chain T, whereby motion is communicated to the truck in one direction or the other, according to the direction of revolution of said pinion S.

130 To temper a tube it is heated in the furnace A to a suitable temperature. A rod is then passed through the center, and a key is in-

4  
stered through the projecting lower end of the rod. The chamber R permits this to be done. The tube is then lifted, and another key is inserted in the rod above the tube. When the tube is out of the former, it is transported above the vessel B, in which the lead bath has been raised to the desired temperature. The drag-chain J is then fastened to the end of the rod V and the tube drawn into the bath, in which it is allowed to remain for the time judged necessary.

5 The precise means described, it will be observed, are not of the essence of the invention. The means for heating and for effecting the immersion can be varied according to the form of the pieces. Moreover, it is not designed to claim herein nor to restrict the claims to the precise means of handling the pieces to be tempered.

- 20 20 I claim as my invention or discovery—  
1. The improvement in tempering or hardening armor-plates, cannon-tubes, and other large objects of that order, consisting in heating the object to or about a cherry-red or orange-yellow, forcing it while thus hot under a tempering-bath of molten metal having an initial temperature of about 400° centigrade, and being of a volume readily comparable with that of the object to be tempered, particularly 25 a bath of molten lead of three or four times the weight of said object, and keeping the said object submerged till it has attained the temperature of the molten-metal bath, so that the tempering or hardening is effected by a comparatively prolonged conduction from the sur-

45 face of the armor-plate, cannon-tube, or other large object of that order to the molten metal in contact therewith, and also through the mass of the said object and of the molten metal, under a surface pressure in excess of that attained by the old use of non-metallic liquids, substantially as described, the specified conditions of temperature and the like being variable more or less, according to the nature of the metal to be tempered, the degree of temper to be produced, and the special circumstances, as the skilled operator may determine, as hereinbefore set forth.

45 50 2. The new and improved apparatus for tempering or hardening armor-plates, cannon-tubes, and other large objects of that order in molten-metal baths, consisting of two furnaces, each provided with means for heating the contents, and one of them containing a molten-metal tempering-bath, and being also provided with means for forcing the large objects to be tempered under the molten metal of the bath and holding them there, and, in connection with said furnaces, of mechanical appliances—such as trucks and lifts—for transferring said 55 large objects to the furnace containing the metal bath from the other of said furnaces, substantially as described.

50 55 In testimony whereof I have signed this specification in the presence of two subscribing 60 witnesses.

65 ALFRED EVRARD.

Witnesses:

J. JANTET,

J. A. COURNIER BILLIO.